

## UNITED STATES PATENT OFFICE

2,359,581

## METHOD OF AND MIXTURE FOR COKING

Horace C. Porter, Philadelphia, Pa.

No Drawing. Application November 26, 1940,  
Serial No. 367,232

3 Claims. (Cl. 202—33)

This invention relates to coking coal, and more particularly to an improved process for coking coal and to an improved coal mixture for coking purposes to improve the quality and yield of the coking operation and to eliminate destructive expansion properties of coking coal.

In carrying out a coking operation bituminous coal is subjected to heat to drive off volatile constituents of the coal and to transform the coal into a form called "coke." The products of the distillation are generally recovered as coke oven gas, tar, ammonia, and other products. The coke itself is used primarily for metallurgical purposes and its physical structure must be so strong that it does not deteriorate in handling nor crush under the weight of the material being treated with the coke. Also, the coke must be sufficiently porous to provide a large contact surface with gases passed through the coke during the process of utilization.

During the coking operation the coal is heated and its temperature is raised to the point where decomposition and distillation of materials making up the coal takes place. At this temperature some of the materials fuse or soften so that the coal becomes a fluid mass. As the volatile constituents form in and escape from this fluid mass, gas pockets form in it and as the heat treatment continues, the mass solidifies in a porous condition. Coal which has the property of thus agglutinating during the heating operation is called "coking coal" and such property is necessary in order to obtain a coke which has a strong physical structure.

The degree of the fluidity of the mass during the coking operation is important and different coals have different degrees of fluidity. As a general rule, the higher the percent of volatile constituents in the coking coal the greater will be its fluidity during the coking operation. If the fluidity is not sufficiently high the gas formed during the coking treatment is not able to pass off freely from the mass and creates a pressure which causes the mass to expand or create expansion pressure, largely sideways, so as to crack, bulge, distort or weaken the walls of the coke oven. Coking coals having such a low fluidity characteristic during coking are called "expansive" coals. Although these coals give a higher percent yield of coke per ton of coal charged (because of the relatively small loss of volatile matter) they are undesirable when coked alone because of the damage they cause to the coke ovens. Hence coking coals having a low percentage (for example 14—23%) of volatile con-

stituents are generally considered as unuseable for coking, except in mixture with contracting coals.

Coking coals having more than a small expansive characteristic are generally mixed with a so-called contracting or "shrinking" coking coal to insure sufficient fluidity to avoid dangerous expansion and to improve coke quality. Such a "shrinking" coal is a coal having a relatively high volatile content, i. e. 28-38% and a correspondingly high fluidity characteristic. The use of this shrinking coal, however, reduces the coke yield per ton of coal charged because of the distillation of the volatile constituents.

15 By the practice of the present invention it is possible to use normally highly expansive coals in coking ovens without damaging the oven and without admixing coals of higher volatile content and greater fluidity. With such use of expansive low volatile coals the quality and yield of the coke is improved.

I have discovered that the normally destructive expansive properties of a low volatile coking coal having a low fluidity characteristic may be 25 eliminated by admixing with it a certain type of naturally altered low-volatile coal that is non-coking (non-agglutinating) or only slightly coking coal and that such a coal mixture gives a high coke yield of good physical structure without damaging the oven walls. Such expansive coals are found in many coal fields such as, for example, the Huntingdon-Broadtop field, Rockhill, and others, in Pennsylvania; several fields in Cambria, Clearfield and Indiana counties in Pennsylvania; in the Pocahontas field and others of West Virginia; and many other fields.

30 Coals of the low-volatile, non-agglutinating (or slightly agglutinating) type are coals which have been weathered or oxidized and so have a higher oxygen content than the usual low-volatile agglutinating coals and have other differences. Such coals are best obtained from coal seams located near the earth surface and subject to infiltration of oxygen from the air. Such non-agglutinating or slightly agglutinating coals, 35 slowly oxidized and altered over a period of many years, are more completely and uniformly oxidized, and, being oxidized without heat and in the presence of moisture, are chemically altered 40 in different fashion through a greater degree of additive oxygenation than are coals artificially oxidized in known ways. Seam-oxidized non-agglutinating or slightly agglutinating coals of 45 this type are found in many coal fields such as, 50 for example, the Huntingdon-Broadtop and

Cambria fields of Pennsylvania, the Pocahontas field of West Virginia, and others.

By way of illustration, a satisfactory coal mixture is 65-50 parts of "underground mine" Rockhill coal (Pennsylvania) with 35-50 parts of seam-oxidized "strip-mined" low-volatile coal taken from a seam 8-20 feet beneath the surface. Such coals have the following analysis:

Rockhill:

Moisture 1.0, volatile 16.0, ash 6.5, sulphur 1.1, oxygen 2.9%.

Seam-oxidized:

Moisture 3.5, volatile 15.7, ash 5.5, sulphur .65, oxygen 6.2%.

Examples of other mixtures are:

(a) 25 parts Pittsburgh-seam, high-volatile coking coal, 55 parts Rockhill (Pennsylvania) low-volatile coking coal, 20 parts seam-oxidized "strip-mine" low-volatile coal;

(b) 75 parts Cambria Co. (Pennsylvania) Lower Kittanning seam, low-volatile coking coal, with 25 parts seam-oxidized Cambria low-volatile coal.

The two coals should be crushed to a size under  $\frac{1}{4}$ " and then blended or mixed in any suitable thorough manner and the mixture charged to coke ovens of the by-product recovery type and coked in the usual manner. The destructive expansion quality of the coking coal is eliminated and the coke obtained has a physical structure superior to that obtained by coking the coking coal alone. It is superior also in many respects to coke obtained from coals or coal mixtures having higher fluidity characteristics and the yield is greater than that obtained from coals of higher volatile content. Further, because oxidized non-agglutinating coals have at equal oven heats a higher rate of coke formation, the coking operation proceeds in a shorter period of time than that required by coking coals or coking coal mixtures of the usual non-oxidized type.

If more volatile matter is desired, as when the coking operation is carried out by coke plants producing coke oven gas for outside sale, a high-volatile coal may be added in suitably regulated amount to the coking and non-coking coal mix-

ture above described. Also heavy petroleum oils may be added to the mixture to increase the distillation products without reducing the coke yield or the quality of the coke.

5 I claim:

1. The method of manufacturing metallurgical coke comprising making a blend consisting of 50-85 parts of a coking coal having a volatile component of 14-23% on a dry ash-free basis and 15-50 parts of a non-coking, or poorly coking, seam-oxidized coal having a volatile content of 15-20% and an oxygen content of 3.6-4.5% on a dry ash-free basis, coking said blend in a by-product oven at temperatures exceeding 900° C. to distill off the by-products and convert the blend into coke.

10 2. The method of manufacturing metallurgical coke comprising making a blend consisting of a low volatile coal having a volatile component of 14-23% on a dry ash-free basis and objectionable expansion characteristics and a non-coking, or poorly coking, seam-oxidized coal having a volatile content of 15-20% and an oxygen content of 3.6-4.5% on a dry ash-free basis, said latter coal being present in sufficient quantity to eliminate the objectionable expansion characteristic of the low volatile coking coal, and coking said blend in a by-product coke oven at temperatures exceeding 900° C. to distill off the by-products and convert the blend into coke.

15 3. The method of manufacturing metallurgical coke comprising making a blend consisting of a low volatile coking coal having a volatile component of 14-23% on a dry ash-free basis and objectionable expansion characteristics and a non-coking, or poorly coking, seam-oxidized coal having a volatile content of 15-20% and an oxygen content of 3.6-4.5% on a dry ash-free basis said seam-oxidized coal being present in an amount sufficient to offset the expansive characteristics of said coking coal, and a coal having a volatile content of 28-35% to increase the by-product yield, and coking said blend in a by-product coke oven at temperatures exceeding 900° C. to distill off the by-products and convert the blend into coke.

40 HORACE C. PORTER.